

SAMUEL S. UTTER.  
Oven-Door for Cooking-Stoves.  
No. 127,718.

Patented June 11, 1872.



Witnesses  
A. M. MacCormack  
John. F. Smith

Inventor  
Samuel Utter

## UNITED STATES PATENT OFFICE.

SAMUEL S. UTTER, OF BROOKLYN, NEW YORK.

## IMPROVEMENT IN OVEN-DOORS OF COOKING-STOVES.

Specification forming part of Letters Patent No. 127,718, dated June 11, 1872.

*To all whom it may concern:*

Be it known that I, SAMUEL S. UTTER, of the city of Brooklyn, State of New York, have invented a new and useful Improvement in Oven-Doors of Stoves, Ranges, or other Cooking Apparatus; and hereby declare that the following is a full and complete description thereof.

In order to better reflect the heat and produce a higher temperature in ovens, it has been the practice to coat the inside of the oven-doors with sheet-tin; but the tin in a short time loses its brightness, and the surface melts off, thereby losing its properties of reflection and becoming useless. My invention consists in providing the inside of oven-doors with a material which will have all the properties of reflection that the bright surface of tin has, and not being as good a conductor of heat as metal, will prevent its escape by absorption, thereby raising the temperature in the oven.

To produce these improved results, I place a layer of enamel on the inside of the oven-door, thus giving a polished surface which will bear a high temperature without tarnishing, and, by its imperfect conducting qualities, prevent the escape of the heat. This may be

done by placing a coating of enamel on the inside surface of the oven-door direct, or by attaching sheets of iron or other material, previously enameled, thereon by means of rivets or other suitable fastenings.

In the drawing, Figure 1 is a view showing the inside surface of the oven-door, and Fig. 2 is a section through Fig. 1 at the dotted line *xx*.

A represents the metallic portion of the oven-door and B the enameled surface thereof. Any color of enamel may be used for this purpose, but I prefer white, as it absorbs less radiant heat than any other color. The enamel also gives to the oven-doors a much better finish, and they can be kept perfectly clean and bright with very little trouble, only needing to be wiped with a cloth, which restores them to their original brightness.

*Claim.*

An oven-door having an enameled inside surface, substantially as described.

SAMUEL S. UTTER.

## Witnesses.

A. B. MALCOMSON, JR.,  
JAMES H. HUNTER.